

# United States Patent [19]

Kato et al.

[11] Patent Number: 4,988,449

[45] Date of Patent: Jan. 29, 1991

[54] FLUID-PERMEABLE AGENT FOR  
NON-WOVEN SHEETS OF POLYOLEFIN  
FIBERS

[75] Inventors: Tomohiro Kato, Nagoya; Yoshio  
Takasu; Makoto Minafuji, both of  
Aichi, all of Japan

[73] Assignee: Takemoto Yushi Kabushiki Kaisha,  
Aichi, Japan

[21] Appl. No.: 400,356

[22] Filed: Aug. 30, 1989

## Related U.S. Application Data

[63] Continuation-in-part of Ser. No. 210,636, Jun. 23, 1988,  
abandoned.

## Foreign Application Priority Data

Jun. 25, 1987 [JP] Japan ..... 62-158162

[51] Int. Cl.<sup>5</sup> ..... D06M 13/10; D06M 13/419;  
D06M 13/473; D06M 13/292

[52] U.S. Cl. ..... 252/8.8; 252/8.7;  
252/8.75; 252/8.6; 252/547; 252/135

[58] Field of Search ..... 252/8.6, 8.75, 8.8,  
252/8.9, 547

## References Cited

### U.S. PATENT DOCUMENTS

3,696,034 10/1970 Hewitt et al. ..... 252/8.8  
3,835,148 9/1974 Oxé et al. ..... 252/8.8  
3,908,048 9/1975 Kawanaka et al. ..... 252/8.8  
3,935,150 1/1976 Oxé et al. ..... 252/8.8

3,956,350 5/1976 Pusch et al. ..... 252/8.8  
3,966,659 6/1976 Oxé et al. ..... 252/8.8  
3,983,061 9/1976 Oxé et al. ..... 252/8.8  
4,076,631 2/1978 Caruso et al. ..... 252/8.8

## OTHER PUBLICATIONS

McCutcheon's Emulsifiers and Detergents, 1983, pp.  
115-116, also pp. 167, 215.

Primary Examiner—Paul Lieberman

Assistant Examiner—J. Darland

Attorney, Agent, or Firm—Flehr, Hohbach, Test,  
Albritton & Herbert

[57]

## ABSTRACT

A fluid-permeable agent for providing fluid-permeability to non-woven sheets of polyolefin fibers contains 50 wt % or more of aliphatic diethanol amide shown by the formula:



where R is alkyl or alkenyl group with 11-17 carbon atoms. The agent may additionally contain non-ionic surfactants and salt of certain specified kinds and is applied at a rate of 0.1-0.5 wt % with respect to the fibers for good results.

5 Claims, No Drawings

## FLUID-PERMEABLE AGENT FOR NON-WOVEN SHEETS OF POLYOLEFIN FIBERS

This is a continuation-in-part, division, of application Ser. No. 210,636 filed June 23, 1988, now abandoned.

### BACKGROUND OF THE INVENTION

This invention relates to fluid-permeable agents for non-woven sheets made of polyolefin fibers such as composite synthetic fibers having sheath-core structure made of two or more polymers with different melting points having polyolefin polymer sheaths and also to application methods of such agents. More particularly, this invention relates to agents to be applied to such fibers for providing durability and fluid-permeability and also to methods of applying such agents.

Recently, non-woven sheets by a dry-bonding process and more particularly bondable non-woven sheets are coming to be frequently used in medical supplies and hygienical articles. For diapers, napkins and the like, polyolefin fibers and composite polyethylene fibers are frequently used in view of their skin-comfortability (that is, softness and absence of discomfort from wetting). In order to improve product characteristics such as bulkiness, restorability and shape-stability against heat, on the other hand, use is frequently made of heat-bondable composite fibers comprised of polyester fibers and polypropylene fibers as the core and polyolefin polymers as the sheath.

In order to eliminate user's discomfort from a diaper, a napkin and the like caused by sweat, urine, menstrual fluid and other body fluids, it is considered important not only that the body-facing parts of these products be wettable but also their wettability can be quickly manifested. For this reason, fluid-permeability within a short time is a required characteristic of polyolefin fibers of which these body-facing parts are comprised. Since diapers, in particular, are generally worn by infants, seniors and very sick persons who cannot take care of themselves, a single diaper should be able to handle two or more discharges without causing discomfort to the wearer. For this reason, durability of fluid-permeability (or durability against repeated use) is another strongly required characteristic.

Prior art methods of providing fluid-permeability to polyolefin fibers and sheaths of polyolefin composite fibers include (1) application of a low-molecular weight hydrophilic compound (U.S. Pat. Nos. 3,664,343 and 3,821,021), (2) application of a hydrophilic macromolecular resin (U.S. Pat. Nos. 3,934,587, 4,297,410, 4,406,660 and 4,718,899), (3) improvement of surface characteristics by chemical processing, solvent processing, plasma processing, corona discharge processing, etc. By the first of the above methods, however, not only desired fluid-permeability cannot be obtained because these agents cannot wet the fiber surface satisfactorily but also there is no durability even if fluid-permeability can be obtained to a certain extent and, in many instances, the user's skin is seriously irritated. The second of the above methods, on the other hand, generally cannot provide sufficient fluid-permeability. Additional disadvantages include insufficiency in durability if use is made of an agent which can provide fluid-permeability to a certain extent. Moreover, agents of this type have the tendency of causing troubles of various kinds during the production process of non-woven sheets. As for the third of the above methods, although it provides rela-

tively favorable results regarding skin-irritation and permeability, resultant fluid-permeability tends to deteriorate with time along with the polar groups which are generated by the surface changes of the fibers. In other words, this method not only provides insufficient durability but also is itself uneconomical.

There have been proposals, on the other hand, to use a hydrophilic polymer as base material and to partially coat its surface with a hydrophobic compound. A water repellent polymer may be used as the hydrophobic compound as disclosed in U.S. Pat. No. 3,934,587. Alternatively, use may be made of a compound of silicon or fluorine as disclosed in U.S. Pat. No. 3,838,692. These proposed methods are equally unsatisfactory because a basically hydrophilic polymer is used as the base material and the aforementioned characteristics of basically hydrophobic polyolefin fibers are lacking.

### SUMMARY OF THE INVENTION

Polyolefin fibers being basically very poor in permeability because of their low surface energy characteristics, it is an object of the present invention to provide fluid-permeable agents for non-woven sheets of polyolefin fibers with which the aforementioned problems of prior art agents can be eliminated.

The present invention has been completed by the present inventors as a result of their diligent studies in view of the aforementioned and other objects and is based on their discovery that desired results are obtainable by agents containing more than a specified amount of specified kinds of aliphatic diethanol amide and also a specified kind of surfactant appropriately selected for the purpose.

### DETAILED DESCRIPTION OF THE INVENTION

Fluid-permeable agents according to the present invention for non-woven sheets of polyolefin fibers are characterized as containing 70-95 wt% of aliphatic diethanol amide shown by the following Formula A:



where R is alkyl or alkenyl group with 11-17 carbon atoms, and 5-30 wt% of surfactant including one or more selected from the following:

(a) non-ionic surfactants each derived from an addition reaction of alkylene oxide with 2-3 carbon atoms to an active hydrogen compound having alkyl or alkenyl group with 11-22 carbon atoms as a hydrophobic group, 3-10 moles of said alkylene oxide being added per hydrophobic group of said active hydrogen compound being added in said addition reaction,

(b) alkyl phosphate salt shown by the following formula:



where  $\text{R}^1$  is alkyl or alkenyl group with 12-18 carbon atoms, M is Na, K or ammonium, and a and b are integers equal to or greater than 1 that  $a+b=3$ ,

(c) quaternary ammonium salt shown by the following formula:



where  $R^1$  is alkyl or alkenyl group with 12-18 carbon atoms,  $R^2$  is H, alkyl or hydroxylalkyl group with 1-2 carbon atoms or  $R^1$ , and  $X$  is halogen, residue of organic or inorganic acid, or alkyl sulfate or alkyl phosphate with 1-2 carbon atoms, and

(d) alkyl imidazolinium salt shown by the following formula:



$R^2$  is H, alkyl or hydroxylalkyl group with 1-2 carbon atoms, or alkyl or alkenyl group with 12-18 carbon atoms,  $X$  is halogen, residue of organic or inorganic acid, or alkyl sulfate or alkyl phosphate with 1-2 carbon atoms,  $R^3$  is alkyl or alkenyl group with 11-17 carbon atoms and  $R^4$  is  $C_2H_4OH$ ,  $C_2H_4NH_2$ ,  $C_2H_4NHCOCH_3$  or  $C_2H_4NHCOR^3$ .

Aliphatic diethanol amides shown by the formula above are compounds which are obtainable generally by reaction between methyl ester of aliphatic acid and diethanol amine. They may be called (1:1) type alkylol amide or (1:2) type alkylol amide, depending on the conditions of the reaction, but their principal constituent is a compound of the structure shown by the formula above.

Regarding the aliphatic diethanol amides described above, the residue of aliphatic acid (or  $R$ ) is limited to alkyl or alkenyl group with 11-17 carbon atoms. With alkyl group or alkenyl group with 18 or more carbon atoms, the resultant aliphatic diethanol amide is less soluble or nearly insoluble in water and not only is it impossible to obtain a stable solution of the agent but a non-woven sheet treated with such an agent does not acquire sufficient permeability. If the alkyl or alkenyl group has less than 11 carbon atoms, on the other hand, durability of processed non-woven sheets becomes extremely poor. If aliphatic diethanol amide is contained by less than 50 wt%, furthermore, both permeability and durability of the processed non-woven sheets become extremely poor. If durability is important with sufficient permeability, in particular, agents containing more than 70 wt% of stearic diethanol amide.

It is preferable to use the aliphatic diethanol amide together with a surfactant of specified kinds in order to improve the characteristics related to the production processes of non-woven sheets without adversely affecting the aforementioned permeability and durability of aliphatic diethanol amide. Among preferable surfactants are non-ionic surfactants derived from an addition reaction of alkylene oxide such as ethylene oxide and propylene oxide to an active hydrogen compound having alkyl or alkenyl group with 11-22 carbon atoms as hydrophobic group wherein 3-10 moles of the alkylene oxide are added per hydrophobic group of the active hydrogen compound. Such a surfactant is preferably

added to an aliphatic diethanol amide at the concentration of about 5-30 wt%. With a non-ionic surfactant having alkyl or alkenyl group with less than 11 carbon atoms, the agent is not uniformly attached to fibers and both its fluid-permeability and durability become poor. The result is approximately the same if the number of carbon atoms exceeds 22. If less than 3 moles of alkylene oxide is added, both solubility into water and stability of solution become poor and abnormal attachment to fibers may occur such that fluid-permeability becomes poorer. If more than 10 moles of alkylene oxide is added, on the other hand, durability of aliphatic diethanol amide is affected.

Examples of preferable non-ionic surfactant include POE(7) stearyl ether, POE(5) oleate ether, PEG(400) stearate, POE(10) lauryl ether stearate, POE(4) cetyl amino ether, POE(7) stearoyl amino ether, ethylene oxide (7 mole) adduct of sorbitan monostearate, trimethylol propane-ethylene oxide (9 mole) adduct of tristearate, ethylene oxide (10 mole) adduct of pentaerythritol distearate, castor oil ethylene oxide (25 moles) adduct of trioleate, and propylene oxide (4 mole) ethylene oxide (6 mole) adduct of stearyl alcohol. In the above and hereinafter, POE and PEG respectively indicate polyoxyethylene and polyethyleneglycol and the numeral inside the parentheses which follow indicates the molar number of addition.

Preferable surfactants of another kind to be used together with the aforementioned aliphatic diethanol amides according to the present invention include alkyl phosphate salts shown by the following general formula (Formula B), quaternary ammonium salts shown by the following general formula (Formula C) and alkyl imidazolinium salts shown by the following general formula (Formula D):



where  $R^1$  is alkyl or alkenyl group with 12-18 carbon atoms,  $M$  is Na, K or ammonium, and  $a$  and  $b$  are integers equal to or greater than 1 such that  $a+b=3$ ;



and



where  $R^1$  is alkyl or alkenyl group with 12-18 carbon atoms,  $R^2$  is H, alkyl or hydroxylalkyl group with 1-2 carbon atoms or  $R^1$ ,  $R^3$  is alkyl or alkenyl group with 11-17 carbon atoms,  $R^4$  is  $C_2H_4OH$ ,  $C_2H_4NH_2$ ,  $C_2H_4NHCOCH_3$  or  $C_2H_4NHCOR^3$ , and  $X$  is halogen, residue of organic or inorganic acid or alkyl sulfate or alkyl phosphate with 1-2 carbon atoms. It is preferable

that these surfactants be contained by 5-30 wt% in the agent of the present invention.

When such (alkyl phosphate, quaternary ammonium and alkyl imidazolinium) salts are used together with the aforementioned aliphatic diethanol amides and non-ionic surfactants of the present invention, it is preferable to mix them together such that the mixture has 70-85 wt% of aliphatic diethanol amide, 5-20 wt% of non-ionic surfactant and 5-15 wt% of one selected from the group consisting of alkyl phosphate salts, quaternary ammonium salts and alkyl imidazolinium salts. The salts of the aforementioned group are capable of improving the processability of non-woven sheets during their production without adversely affecting the fluid-permeability and durability of aliphatic diethanol amides. In particular, antistatic characteristics, card-processability and uniformity of web during a web-formation process can be obtained with them. The limiting conditions presented above with respect to these salts are important, for example, in that those with smaller alkyl or 15 alkenyl groups than specified above adversely affect the durability of aliphatic diethanol amides and that those with larger alkyl or alkenyl groups than specified above tend to obstruct the fluid-permeability of aliphatic diethanol amides. Examples of ammonium in Formula B 25 include  $\text{NH}_4$ ,  $\text{NH}(\text{CH}_3)_3$ ,  $\text{NH}(\text{C}_2\text{H}_5)_3$ ,  $\text{NH}_2(\text{CH}_2\text{CH}_2\text{OH})_2$  and  $\text{NH}(\text{CH}_2\text{CH}_2\text{OH})_3$ .

Composite fibers with a sheath part of polyethylene polymer and a core part of polypropylene or polyester fibers are representative examples of polyolefin fibers to which the fluid-permeable agents of the present invention are applicable but the present invention is by no means limited to application to such fibers. The agents of the present invention are also applicable not only to composite fibers in general with a sheath part of polyolefin polymer and a core part of another polymer with a different melting point but also to polyethylene fibers, polypropylene fibers and other copolymer fibers not by composite spinning.

The agents of the present invention should preferably be applied to such polyolefin fibers generally at the rate (with respect to the fibers) of 0.05-0.7 wt% and more preferably 0.1-0.5 wt%. Methods of application include dipping, spraying and the roller-touch method. The polyolefin fibers to which an agent has been applied is 45 dried for production of non-woven sheets by card processing and heat bonding.

In what follows, examples of tests and their results are presented to further describe the present invention but it goes without saying that these examples are not 50 intended to limit the scope of the invention. For testing, agents inclusive of eight test examples and six comparison examples were prepared with constituents selected as follows and shown in Table 1:

Test Example 1 comprising 80 wt% of stearic diethanol amide (reaction product of methyl stearate and diethanol amide) and 20 wt% of lauric diethanol amide (reaction product of methyl stearate and diethanol amide); Test Example 2 comprising 90 wt% of stearic diethanol amide and 10 wt% of polyethylene oxide (4 60 mole) condensate of octylalcohol; Test Example 3 comprising 70 wt% of stearic diethanol amide and 30 wt% of polyethylene oxide (7 mole) condensate of stearic amide; Test Example 4 comprising 50 wt% of stearic diethanol amide and 50 wt% of PEG (molecular weight 65 about 300) monostearate; Test Example 5 comprising 70 wt% of stearic diethanol amide and 30 wt% of tristearate of polyethoxylated (24 mole) glycerin; Test Exam-

ple 6 comprising 75 wt% of stearic diethanol amide, 10 wt% of polyethylene oxide (7 mole) condensate of stearic amide and 15 wt% of potassium stearyl phosphate; Test Example 7 comprising 70 wt% of stearic diethanol amide, 20 wt% of polyethylene oxide (7 mole) condensate of stearic amide and 10 wt% of 1-(2-hydroxyethyl)-1-ethyl-2-heptadecyl-2-imidazolinium ethyl sulfate; Test Example 8 comprising 80 wt% of stearic diethanol amide, 15 wt% of polyethylene oxide (10 mole) condensate of stearyl alcohol and 5 wt% of distearyl dimethyl ammonium chloride; Comparison Example 1 being sodium dioctyl sulfosuccinate; Comparison Example 2 being potassium cetyl phosphate; Comparison Example 3 being polymeric condensates of dimethyl terephthalate, dimethyl isophthalate and PEG (molecular weight about 10,000); Comparison Example 4 comprising 40 wt% of stearic diethanol amide and 60 wt% of polyethylene oxide (10 mole) condensate of lauryl alcohol; Comparison Example 5 comprising 70 wt% of behenic diethanol amide and 30 wt% of polyethylene oxide (7 mole) condensate of stearic amide; and Comparison Example 6 comprising 70 wt% of lauric monoethanol amide and 30 wt% of polyethylene oxide (7 mole) condensate of stearic amide. Samples with 0.2 wt% of agents were prepared by dipping composite fibers of 2 denier  $\times$  51 mm cut length with sheath part of polyethylene and core part of polyester in 1.0% solution of each of the agents listed in Table 1 for two minutes at 40° C., thereafter squeezing to 20 wt% and wind-drying for 60 minutes at 60° C.

Antistatic characteristics of the samples were evaluated by keeping them for 24 hours under temperature-humidity conditions of 25° C. and 40%RH and measuring the generated voltage as they were passed through an opener and a roller card under these conditions such that the web weight became 24g/m<sup>2</sup>. The results of the measurements are shown in Table 2.

TABLE 1

| Classification | Component                                                                     | Content (wt %) |
|----------------|-------------------------------------------------------------------------------|----------------|
| Example 1      | $\text{C}_2\text{H}_4\text{OH}$                                               | 80             |
|                | $\text{C}_{17}\text{H}_{35}\text{CON}$                                        |                |
|                | $\text{C}_2\text{H}_4\text{OH}$                                               | 20             |
|                | $\text{C}_2\text{H}_4\text{OH}$                                               |                |
| Example 2      | $\text{C}_2\text{H}_4\text{OH}$                                               | 90             |
|                | $\text{C}_{17}\text{H}_{35}\text{CON}$                                        |                |
|                | $\text{C}_2\text{H}_4\text{OH}$                                               |                |
|                | $\text{C}_8\text{H}_{17}\text{O}-(\text{CH}_2\text{CH}_2\text{O})_4-\text{H}$ | 10             |
| Example 3      | $\text{C}_2\text{H}_4\text{OH}$                                               | 70             |
|                | $\text{C}_{17}\text{H}_{35}\text{CON}$                                        |                |
|                | $\text{C}_2\text{H}_4\text{OH}$                                               |                |
|                | Polyethylene oxide (7 mole) condensate of stearic amide                       | 30             |
| Example 4      | $\text{C}_2\text{H}_4\text{OH}$                                               | 50             |
|                | $\text{C}_{17}\text{H}_{35}\text{CON}$                                        |                |
|                | $\text{C}_2\text{H}_4\text{OH}$                                               |                |
|                | PEG (molecular weight about 300) monostearate                                 | 50             |

TABLE 1-continued

| Classification | Component                                                                                                                                                                                                                                                                                                                                                                                                | Content (wt %) |                                              |
|----------------|----------------------------------------------------------------------------------------------------------------------------------------------------------------------------------------------------------------------------------------------------------------------------------------------------------------------------------------------------------------------------------------------------------|----------------|----------------------------------------------|
| Example 5      | $\begin{array}{c} \text{C}_2\text{H}_4\text{OH} \\   \\ \text{C}_{11}\text{H}_{23}\text{CON} \\   \\ \text{C}_2\text{H}_4\text{OH} \\   \\ \text{C}_{17}\text{H}_{35}\text{CO}-(\text{OC}_2\text{H}_4)_8-\text{OCH}_2 \\   \\ \text{C}_{17}\text{H}_{35}\text{CO}-(\text{OC}_2\text{H}_4)_8-\text{OCH}_2 \\   \\ \text{C}_{17}\text{H}_{35}\text{CO}-(\text{OC}_2\text{H}_4)_8-\text{OCH}_2 \end{array}$ | 70             | 5                                            |
|                |                                                                                                                                                                                                                                                                                                                                                                                                          | 30             | 5<br>6<br>7<br>8                             |
|                |                                                                                                                                                                                                                                                                                                                                                                                                          | 10             | 12<br>22<br>10<br>21                         |
|                |                                                                                                                                                                                                                                                                                                                                                                                                          |                | 33<br>26<br>14<br>30                         |
|                |                                                                                                                                                                                                                                                                                                                                                                                                          |                | 43<br>29<br>20<br>37                         |
| Example 6      | $\begin{array}{c} \text{C}_2\text{H}_4\text{OH} \\   \\ \text{C}_{17}\text{H}_{35}\text{CON} \\   \\ \text{C}_2\text{H}_4\text{OH} \\   \\ \text{Polyethylene oxide (7 mole)} \\ \text{condensate of stearic amide} \\   \\ \text{Potassium stearyl phosphate} \end{array}$                                                                                                                              | 75             | 15                                           |
|                |                                                                                                                                                                                                                                                                                                                                                                                                          | 10             | 1<br>2<br>3<br>4<br>5<br>6                   |
|                |                                                                                                                                                                                                                                                                                                                                                                                                          | 15             | -0.4<br>+0.8<br>+1.2<br>-0.5<br>+4.0<br>+0.6 |
|                |                                                                                                                                                                                                                                                                                                                                                                                                          |                | 20<br>60≤<br>47<br>24<br>60≤<br>26           |
|                |                                                                                                                                                                                                                                                                                                                                                                                                          |                | 60≤<br>—<br>—<br>—<br>—<br>—                 |
| Example 7      | $\begin{array}{c} \text{C}_2\text{H}_4\text{OH} \\   \\ \text{C}_{17}\text{H}_{35}\text{CON} \\   \\ \text{C}_2\text{H}_4\text{OH} \\   \\ \text{Polyethylene oxide (7 mole)} \\ \text{condensate of stearic amide} \\   \\ 1-(2\text{-hydroxyethyl})-1\text{-ethyl-} \\ 2\text{-heptadecyl-2-imidazolinium} \end{array}$                                                                                | 70             | 20                                           |
|                |                                                                                                                                                                                                                                                                                                                                                                                                          | 20             | 10                                           |
|                |                                                                                                                                                                                                                                                                                                                                                                                                          | 25             | 20<br>60≤<br>—<br>—<br>—<br>—                |
| Example 8      | $\begin{array}{c} \text{C}_2\text{H}_4\text{OH} \\   \\ \text{C}_{17}\text{H}_{35}\text{CON} \\   \\ \text{C}_2\text{H}_4\text{OH} \\   \\ \text{Polyethylene oxide (10 mole)} \\ \text{condensate of stearyl alcohol} \\   \\ \text{Distearyl dimethyl ammonium chloride} \end{array}$                                                                                                                  | 80             | 30                                           |
| Comparison 1   | Sodium sulfosuccinate                                                                                                                                                                                                                                                                                                                                                                                    | 5              | 35                                           |
| Comparison 2   | Potassium cetyl phosphate                                                                                                                                                                                                                                                                                                                                                                                | 100            |                                              |
| Comparison 3   | Polymeric condensates of dimethyl terephthalate, dimethyl isophthalate and PGE (molecular weight about 10,000)                                                                                                                                                                                                                                                                                           | 100            |                                              |
| Comparison 4   | $\begin{array}{c} \text{C}_2\text{H}_4\text{OH} \\   \\ \text{C}_{17}\text{H}_{35}\text{CON} \\   \\ \text{C}_2\text{H}_4\text{OH} \\   \\ \text{C}_{12}\text{H}_{25}\text{O}-(\text{CH}_2\text{CH}_2\text{O})_{10}-\text{H} \end{array}$                                                                                                                                                                | 40             | 40                                           |
| Comparison 5   | $\begin{array}{c} \text{C}_2\text{H}_4\text{OH} \\   \\ \text{C}_{21}\text{H}_{43}\text{CON} \\   \\ \text{C}_2\text{H}_4\text{OH} \end{array}$                                                                                                                                                                                                                                                          | 70             | 45                                           |
|                | Polyethylene oxide (7 mole) condensate of stearic amide                                                                                                                                                                                                                                                                                                                                                  | 30             |                                              |
| Comparison 6   | $\begin{array}{c} \text{C}_2\text{H}_4\text{OH} \\   \\ \text{C}_{11}\text{H}_{23}\text{CON} \\   \\ \text{H} \end{array}$                                                                                                                                                                                                                                                                               | 70             | 50                                           |
|                | Polyethylene oxide (7 mole) condensate of stearic amide                                                                                                                                                                                                                                                                                                                                                  | 30             | 55                                           |

TABLE 2

| Example | Voltage Generated (kV) | Permeability (sec) | Durability |       |                      | Total Number of repetitions |
|---------|------------------------|--------------------|------------|-------|----------------------|-----------------------------|
|         |                        |                    | Once       | Twice | After Each Use (sec) |                             |
| 1       | -0.3                   | 4                  | 20         | 37    | 46                   | 6                           |
| 2       | -0.6                   | 8                  | 15         | 23    | 55                   | 5                           |
| 3       | -0.3                   | 13                 | 9          | 11    | 22                   | 10                          |
| 4       | -0.2                   | 4                  | 16         | 35    | 51                   | 4                           |

TABLE 2-continued

| Voltage Generated (kV) | Permeability (sec) | Durability |       |                      | Total Number of repetitions |
|------------------------|--------------------|------------|-------|----------------------|-----------------------------|
|                        |                    | Once       | Twice | After Each Use (sec) |                             |
| 5                      | 3                  | 12         | 33    | 43                   | 4                           |
| 6                      | 14                 | 22         | 26    | 29                   | 8                           |
| 7                      | 5                  | 10         | 14    | 20                   | 12                          |
| 8                      | 8                  | 21         | 30    | 37                   | 6                           |

For evaluation of fluid-permeability, non-woven sheet samples were prepared by cutting the aforementioned card web to 10 cm × 10 cm and thermally testing for 30 seconds by a heater plate of 130° C. After these sheet samples were conditioned for 24 hours within a chamber at 20° C. and 60 % RH, they were placed on a horizontal plate, water drops of 0.4 ml were dropped from a height of 10 mm and the time required for each water drop to be completely absorbed was measured. The results obtained are also shown in Table 2.

For evaluating durability, after 80 ml of ion exchange water was sprayed over the sample to be passed therethrough, the samples were wind-dried for 90 minutes at 40° C. and the evaluation of fluid-permeability was repeated. If the measured time was 60 seconds or less, it was recorded and the process described above was repeated. The total number of repetitions was also recorded. The results are additionally shown in Table 2.

Table 2 clearly shows that the agents according to the present invention can provide superior fluid-permeability and durability to non-woven sheets made from polyolefin fibers and improve processability of such non-woven sheets during their production.

What is claimed is:

1. A fluid-permeable agent for providing fluid-permeability to non-woven sheets of polyolefin fibers, said agent containing  
70-95 wt% of aliphatic diethanol amide shown by the following formula:



where R is alkyl or alkenyl group with 11-17 carbon atoms, and  
5-30 wt% of surfactant including one or more selected from the following:

- non-ionic surfactants each derived from an addition reaction of alkylene oxide with 2-3 carbon atoms to an active hydrogen compound having alkyl or alkenyl group with 11-22 carbon atoms as a hydrophobic group, 3-10 moles of said alkylene oxide being added per hydrophobic group of said active hydrogen compound being added in said addition reaction,
- alkyl phosphate salt shown by the following formula:



(B)

5

where  $R^1$  is alkyl or alkenyl group with 12-18 carbon atoms, M is Na, K or ammonium, and a and b are integers equal to or greater than 1 such that  $a+b=3$ ,

(c) quaternary ammonium salt shown by the following formula:

15

(C)



where  $R^1$  is alkyl or alkenyl group with 12-18 carbon atoms,  $R^2$  is H, alkyl or hydroxyalkyl group with 1-2 carbon atoms or  $R^1$ , and X is halogen, residue of organic or inorganic acid, or alkyl sulfate or alkyl phosphate with 1-2 carbon atoms, and

(d) alkyl imidazolinium salt shown by the following formula:



(D)

$R^2$  is H, alkyl or hydroxyalkyl group with 1-2 carbon atoms, or alkyl or alkenyl group with 12-18 carbon atoms, X is halogen, residue of organic or inorganic acid, or alkyl sulfate or alkyl phosphate with 1-2 carbon atoms,  $R^3$  is alkyl or alkenyl group with 11-17 carbon atoms and  $R^4$  is  $C_2H_4OH$ ,  $C_2H_4NH_2$ ,  $C_2H_4NHCOCH_3$  or  $C_2H_4NHCOR^3$ .

2. The agent of claim 1 wherein said aliphatic diethanol amide shown by said formula A is stearic diethanol amide.
3. The agent of claim 1 characterized as containing 70-85 wt% of said aliphatic diethanol amide, 5-20 wt% of said non-ionic surfactant and 5-15 wt% of said alkyl phosphate salt.
4. The agent of claim 1 characterized as containing 70-85 wt% of said aliphatic diethanol amide, 5-20 wt% of said non-ionic surfactant and 5-15 wt% of said quaternary ammonium salt.
5. The agent of claim 1 characterized as containing 70-85 wt% of said aliphatic diethanol amide, 5-20 wt% of said non-ionic surfactant and 5-15 wt% of said alkyl imidazolinium salt.

\* \* \* \* \*

35

40

45

50

55

60

65